# EUROPEAN PATENT SPECIFICATION

(11) **EP 0 792 390 B1**
(45) Date of publication and mention of the grant of the patent: **08.03.2000**
(21) Application number: 95942809.5
(22) Date of filing: 15.12.1995
(51) Int. Cl.: C23C 30/00, C04B 41/87, B23B 27/14

(54) **COATED CEMENTED CARBIDE INSERT FOR METAL CUTTING APPLICATIONS**
BESCHICHTETE SINTERKARBIDEINSÄTZE FÜR DIE VERWENDUNG BEIM METALLSCHNEIDEN
INSERT EN CARBURE FRITTE REVETU POUR APPLICATIONS DE COUPE DE METAL

(30) Priority: 30.12.1994 SE 9404587
(43) Date of publication of application: 03.09.1997
(73) Proprietor: SANDVIK AKTIEBOLAG, 811 81 Sandviken (SE)
(72) Inventor: MIKUS, Marian, S-127 37 Skärholmen (SE)
(74) Representative: Östlund, Alf Olof Anders
(86) International application number: SE9501516
(87) International publication number: WO9621052

(56) References cited:
- WO-A-80/02569
- WO-A-92/13112
- GB-A- 2 112 415
- US-A- 4 497 660
- US-A- 4 610 931
- PATENT ABSTRACTS OF JAPAN, Vol. 10, No. 276, C-373; & JP,A,61 096 072 (MITSUBISHI METAL CORP), 14 May 1986.
- PATENT ABSTRACTS OF JAPAN, Vol. 16, No. 334, C-964; & JP,A,04 099 245 (SUMITOMO ELECTRIC IND LTD), 31 March 1992.
- PATENT ABSTRACTS OF JAPAN, Vol. 9, No. 160, C-289; & JP,A,60 033 353 (MITSUBISHI KINZOKU K.K.), 20 February 1985.

## Description

The present invention relates to coated cemented carbide inserts with improved cutting properties being obtained as a result of modifications of the chemical and mechanical properties of the binder phase.

Cemented carbide grades for metal cutting applications generally contain WC, γ-phase (a solid solution of generally TiC, NbC, TaC and WC) and binder phase, generally cobalt. Their properties are optimized by varying the WC grain size, volume fraction of the binder phase and/or the γ-phase and by optimising the carbon content. One recent major improvement of the properties of coated cemented carbide is the introduction of binder phase enriched surface zones.

Thus, two major groups of coated cemented carbide inserts for metal cutting are used today: one with even distribution of binder phase within the whole insert and one with binder phase enriched surface zones.

The cemented carbides with binder phase enriched surface zones are mainly found in γ-phase containing grades whereas straight WC-Co grades have even binder phase distribution without said binder phase enrichment.

In both these groups of cemented carbides the binder phase is based on cobalt containing varying amounts of tungsten and carbon in solid solution. In addition to tungsten or carbon, only very low contents of other elements (mainly impurities) are present in the binder phase.

In applications in highly corrosive environments e.g. wear parts in pumps, compressors or cutters in wood working industry ordinary WC-Co based cemented carbides fail due to corrosion attacks from various types of the corrosive media which react with and deteriorate the cobalt binder phase. In such applications binder phase alloys based on Co-Ni-Cr or Ni-Cr are used e.g. such as disclosed in EP-A-28620.

Surprisingly it has now been found that by using a cemented carbide with a corrosion resistant binder phase large improvements in tool life are achieved for coated cemented carbides in certain metal cutting operations.

The invention relates to a coated cemented carbide for interrupted machining of steel and cast iron metal cutting applications. Said cemented carbide contains 4-14 weight-% binder phase consisting of in solid solution in weight-%: Co 20-80, Mo 1-6, preferably about 2, Cr 3-15, and rest Ni and, optionally W max 30, Mo max 15, Al max 2 and Fe max 70. V may be added up to 5 weight-%.

The Co:Ni weight ratio in the binder phase is about 1:1 or about 3:1.

The carbon content should be between a lower value corresponding to the η-phase limit and an upper value corresponding to the stoichiometric carbon content. In certain embodiments the carbon content can be below the η-phase limit and thus the cemented carbide will contain also η-phase or other substoichiometric phases. 1-20 volume-% has been found suitable.

At too high carbon or chromium contents the brittle chromium carbide is formed and, thus, both chromium and carbon contents must be selected so that the formation of chromium carbide is kept at a minimum.

The invention can be applied to inserts with even distribution of binder phase or, preferably, to inserts with a binder phase enriched surface zone up to 50 µm. The degree of the binder phase enrichment shall be between 1.2 and 2.5 times, preferably between 1.4 and 1.8, higher than the binder phase content of the rest of the insert. Such inserts can be made e.g. using the technique disclosed in US 4,610,931.

The cemented carbide is coated with wear resistant layers as known in the art using known CVD, MTCVD or PVD technique. MTCVD is a moderate temperature CVD-process using e.g. CH₃CN gas and TiCl₄. If the total nickel content is more than about 1.5 weight-% care has to be taken to avoid the detrimental effects of nickel on the coating quality e.g. by using at least at the beginning of the coating process a rather low temperature, preferably <960 °C.

Coatings comprising carbides and/or carbonitrides and/or oxicarbides and/or oxinitrides and/or oxicarbonitrides of titanium and/or Al₂O₃ are particularly useful. In a preferred embodiment at least one 0.3-5 µm, preferably 0.5-1.5 µm, interlayer comprising Ti(C,O) or Ti(C,O,N) or Ti(N,O) is deposited within a part of the coating containing titanium about 0.5-3 µm from the cemented carbide surface such as disclosed in Swedish Patent Application 9400951-1.

The coating thickness shall be 3-16 µm. For milling applications the total coating thickness should be 3-7 µm and for turning applications the total coating thickness should be 5-16 µm.

The present invention is particularly useful in machining of steel and cast iron when the cutting inserts are subjected to thermal and mechanical fatigue conditions. This is typical for milling operations but sometimes it also occurs in certain turning operations with intermittent character.

The reason for the observed tool life for the coated cemented carbide according to the present invention is still not understood in detail. It is believed that through the cracks already present in the coating, or formed during the cutting within the cemented carbide or the coating, the binder phase is oxidised causing weakening of the areas close to the coating. By use of the more oxidation resistant binder phase compositions this type of drawback is largely decreased. The chromium addition increases the binder phase oxidation resistance. However, addition of nickel both increases the oxidation resistance of the cobalt binder phase but also decreases the deformation hardening by stabilization of the FCC-structure of the cobalt phase.

The invention has been described with reference to cutting tool inserts of cemented carbide. It is obvious that the invention can be applied to coated cutting tool insert for metal cutting applications containing at least one hard constituent of a carbide, nitride and/or carbonitride of the metals Ti, Ta, Hf, Nb, V, Zr and W or solid solutions thereof in a binder phase.

### Example 1

Cutting tool inserts according to the invention with the following composition in weight-%: 91.5 WC, 3.9 Co, 3.7 Ni, 0.8 Cr, 0.1 Mo were prepared and coated with a coating consisting of 0.5 µm TiN, 5 µm Ti(C,N) and 3 µm Al₂O₃. The TiN layer was the inner layer closest to the cemented carbide and it was deposited at a temperature of 920 °C. The Ti(C,N) layer was deposited using MTCVD technique.

As reference, inserts with the composition in weight-%: 91.5 WC and 8.5 Co and provided with the same coating were used.
Cutting test:
50 inserts from each group were tested with the following conditions:
Operation: Face milling
Work piece: Pump house in grey cast iron (SS0125)
Cutting speed: 263 m/min
Feed rate: 0.14 mm/tooth
Depth of cut: 2 mm
Cutting fluid: Emulsion
Insert type: TNHF 1204AN-65

Tool life criterion: Edge frittering of the work piece.
Tool life:
Inserts according to the invention: 29 minutes Reference inserts: 16 minutes

### Example 2

Cutting tool inserts according to the invention with the following composition in weight-%: 94.5 WC, 3.3 Co, 1.1 Ni, 0.6 Cr, 0.1 Mo, 0.2 VC were prepared and coated with a coating consisting of: 1.5 µm TiC, 0.5 µm Ti(C,O), 7 µm Ti(C,N) and 6 µm Al₂O₃. The TiC layer was the innermost layer closest to the cemented carbide and the Al₂O₃ layer was the outermost layer.

As reference, inserts with the composition in weight-%: 94.7 WC and 5.3 Co and provided with the same coating were used.
Cutting test.
Operation: Facing with interrupted cuts
Work material: Ferritic-perlitic nodular cast iron (SS0727)
Cutting speed: 150 m/min
Feed rate: 0.1 mm/rev
Depth of cut: 2.0 mm
Cutting fluid: none
Insert type: CNMA 120412
Tool life criterion: Flank wear ≥ 0.3 mm
Tool life:
Inserts according to the invention: 75 min
Reference inserts: 41 min

## Claims

1. Coated insert for interrupted machining of steel and cast iron consisting of a 3-16 µm thick coating comprising at least one carbide or carbonitride or oxicarbide or oxinitrides or oxicarbonitrides of titanium or Al₂O₃ and a substrate containing at least one hard constituent of a carbide, nitride and/or carbonitride of the metals Ti, Ta, Hf, Nb, V, Zr and W or solid solutions thereof in 4-14 weight-% binder phase wherein the binder phase consists of in solid solution the following elements in weight-%: Co 20-80, Cr 3-15, Mo 1-6 and optionally W max 30, Al max 2, Fe max 70 and V up to 5 and rest Ni whereby the Co:Ni weight ratio is about 1:1 or about 3:1.

2. Coated insert according to claim 1 **characterised** in an up to 50 µm thick binder phase enriched surface zone.

3. Coated insert according to claims 1 or 2 **characterised** in that said coating contains at least one 0.3-5 µm layer of Ti(C,O), Ti(C,O,N) or Ti(N,O) about 0.5-3 µm from the substrate surface.

4. Coated insert according to any of the preceding claims **characterised** in containing 1-20 volume-% η-phase or other substoichiometric phase.

## Patentansprüche

1. Beschichteter Einsatz für unterbrochene Bearbeitung von Stahl und Gußeisen, bestehend aus einer 3 bis 16 pm dicken Beschichtung, die wenigstens ein Carbid oder Carbonitrid oder Oxycarbid oder Oxynitrid oder Oxycarbonitrid von Titan oder Al₂O₃ umfaßt, und einem Substrat, welches wenigstens einen harten Bestandteil aus der Gruppe der Carbide, Nitride und/oder Carbonitride der Metalle Ti, Ta, Hf, Nb, V, Zr und W oder feste Lösungen hiervon in 4 bis 14 Gew.-% Bindephase enthält, worin die Bindephase in fester Lösung aus den folgenden Elementen in Gew.-% besteht: Co 20-80, Cr 3-15, Mo 1-6 und gegebenenfalls W maximal 30, Al maximal 2, Fe maximal 70 und V bis zu 5 und Rest Nickel, wobei das Gewichtsverhältnis von Co : Ni etwa 1 : 1 oder 3 : 1 beträgt.

2. Beschichteter Einsatz nach Anspruch 1, gekennzeichnet durch eine bis zu 50 µm dicke Oberflächenzone, die mit Bindephase angereichert ist.

3. Beschichteter Einsatz nach Anspruch 1 oder 2, dadurch gekennzeichnet, daß die Beschichtung wenigstens eine 0,3 bis 5 µm dicke Schicht von Ti(C, O), Ti(C, O, N) oder Ti(N, O) etwa 0,5 bis 3 µm von der Substratoberfläche aus enthält.

4. Beschichteter Einsatz nach einem der vorausgehenden Ansprüche, dadurch gekennzeichnet, daß er 1 bis 20 Vol.-% η-Phase oder andere unterstöichiometrische Phase enthält.

## Revendications

1. Insert revêtu destiné à l'usinage discontinu d'acier et de fonte, constitué d'un revêtement d'une épaisseur de 3 à 16 µm comprenant au moins un élément parmi un carbure ou un carbonitrure ou un oxycarbure ou des oxynitrures ou des oxycarbonitrures de titane ou Al₂O₃, et d'un substrat contenant au moins un constituant dur d'un carbure, nitrure et/ou carbonitrure des métaux Ti, Ta, Hf, Nb, V, Zr et W ou bien des solutions solides de ceux-ci à une concentration en poids de 4 à 14 % de phase liante, dans lequel la phase liante est constituée, en solution solide, des éléments suivants en pourcentage en poids : Co 20 à 80, Cr 3 à 15, Mo 1 à 6 et, optionnellement, W 30 au maximum, Al 2 au maximum, Fe 70 au maximum et V jusqu'à 5, et le reste de Ni, le rapport en poids Co:Ni étant d'environ 1:1 ou d'environ 3:1.

2. Insert revêtu selon la revendication 1, caractérisé par une zone de surface enrichie en phase liante d'une épaisseur allant jusqu'à 50 µm.

3. Insert revêtu selon les revendications 1 ou 2, caractérisé en ce que ledit revêtement contient au moins une couche de 0,3 à 5 µm de Ti(C,O), de Ti(C,O,N) ou de Ti(N,O) à une profondeur de 0,5 à 3 µm depuis la surface du substrat.

4. Insert revêtu selon l'une quelconque des revendications précédentes, caractérisé en ce qu'il contient 1 à 20 % en volume de phase η ou d'une autre phase en dessous de la stoechiométrie.
